

## UNITED STATES PATENT OFFICE.

GEORGE ARTHUR MITCHELL, ARTHUR JAMES MITCHELL, AND ERNEST EDWIN MITCHELL, OF LONDON, ENGLAND, ASSIGNORS TO THE ROADAMANT COMPANY, LIMITED, OF LONDON, ENGLAND.

## CONSTRUCTION OF ROADWAYS, FOOTWAYS, AND THE LIKE.

No. 923,195.

Specification of Letters Patent.

Patented June 1, 1909.

Application filed February 16, 1909. Serial No. 478,168.

To all whom it may concern:

Be it known that we, GEORGE ARTHUR MITCHELL, of 192 Barry Road, East Dulwich, London S. E., England, builder, ARTHUR

5 JAMES MITCHELL, of The Willows, Station Road, Crayford, London, England, quantity-clerk, and ERNEST EDWIN MITCHELL, of 80 Henslowe Road, East Dulwich, London, S. E., England, builder, have invented cer-  
10 tain new and useful Improvements Relating to the Construction of Roadways, Footways, and the Like, of which the following is a specification.

This invention relates to roadways, foot-  
15 ways, courtyards, tennis courts, stair heads, landings, and the like and has for object to provide a durable, dustless and non-slip-  
perly facing or covering capable of with-  
standing extremes of heat and cold.

20 In the specification of previous Letters Patent No. 876377 dated January 14, 1908 we described a method of producing a road or like surface of such a general nature by heating certain constituents therein speci-  
25 fied together with soda and applying the mass in the plastic condition to form the sur-  
face of the road or the like.

As the result of extensive experimen-  
30 tation upon the composition of the prior pat-  
ent we have found that it is possible to obtain a product which is superior to that of said patent in a marked and unexpected degree, by employing the materials and proportions following which must not be  
35 substantially departed from:

|                                                                                                                                      |       |       |
|--------------------------------------------------------------------------------------------------------------------------------------|-------|-------|
| Fine hard stone, e. g. finely broken granite                                                                                         | 30.   | parts |
| Asphalt                                                                                                                              | 58.75 | "     |
| Bitumen                                                                                                                              | 1.25  | "     |
| Hydraulic cement, e. g. Portland                                                                                                     | 7.4   | "     |
| Soda, (i. e. ordinary washing soda, crystal-<br>ized carbonate)                                                                      | .5    | "     |
| 40 Chalk or other mineral carbonate and friable<br>gritty material, e. g. cockle shell or breeze-<br>To which may be added, asbestos | 2.9   | "     |
|                                                                                                                                      | .1    | "     |
|                                                                                                                                      | 100.0 |       |

The bitumen should be first heated in a  
45 caldron, the asphalt then added, and as soon as this has become thoroughly melted the broken granite or fine stone is introduced and intimately mixed with the molten mass. The cement, asbestos, soda, chalk and shell  
50 or breeze, previously well mixed, are now added and the mixture is well stirred, raised to boiling point and allowed to sim-

mer. The mixture can now be placed di-  
rectly on to the road or other surface or it  
may be run into molds and allowed to cool, 55  
and in this latter case it is remelted when  
required for use.

The broken granite or fine stone need not necessarily be mixed with the molten composition in the first instance. In some cases 60 for convenience of transport or otherwise, the stone may be mixed with the other ingredients by remelting these at the place where the covering is to be laid. In some cases also the soda may be added last and 65 stirred in when the mass is thoroughly melted.

As above indicated other hard stone of the district, say flint, may be used instead of granite, and in place of chalk another mineral carbonate such as magnesian limestone or dolomite may be used. Moreover the asbestos may in some cases be safely omitted.

When the material has been laid in mastic form the soft surface is preferably sprinkled 75 with sand, which is rubbed in, and this rubbing process incidentally removes any blow-holes which may form on the surface.

What we claim and desire to secure by Letters Patent is:—

1. A covering for roadways or other sur-  
faces comprising fine stone, asphalt, bitu-  
men, hydraulic cement, soda, mineral car-  
bonate and friable gritty material in ap-  
proximately the relative proportions of 3000 85  
parts of the first, 5875 parts of the second,  
125 parts of the third, 740 parts of the  
fourth, 50 parts of the fifth and 200 parts  
together of the sixth and seventh, substan-  
tially as described.

2. A covering for roadways or other sur-  
faces consisting of fine stone, asphalt bitu-  
men, hydraulic cement, soda, asbestos, min-  
eral carbonate and friable gritty material in approximately the relative proportions of 95  
3000 parts of the first, 5875 parts of the sec-  
ond, 125 parts of the third, 740 parts of the  
fourth, 50 parts of the fifth, 10 parts of the  
sixth and 200 parts together of the seventh  
and eighth, substantially as described.

3. A covering for roadways or other sur-  
faces, consisting of fine stone, as broken  
granite, 3000 parts, asphalt 5875 parts, bitu-  
men 125 parts, Portland cement, 740 parts,

soda 50 parts, chalk and shell together 200 parts.

4. A covering for roadways or other surfaces, consisting of fine stone, as broken granite, 3000 parts, asphalt 5875 parts, bitumen 125 parts, Portland cement, 740 parts, soda 50 parts, chalk and shell together 200 parts, and asbestos 10 parts.

In witness whereof, we have hereunto

signed our names in the presence of two subscribing witnesses.

GEORGE ARTHUR MITCHELL.  
ARTHUR JAMES MITCHELL.  
ERNEST EDWIN MITCHELL.

Witnesses:

FREDERICK WILLIAM BEUER,  
ROBERT MILTON SPEARPOINT.

*No references.*